



US007163657B2

(12) **United States Patent**  
**Heinrich et al.**

(10) **Patent No.:** **US 7,163,657 B2**  
(45) **Date of Patent:** **Jan. 16, 2007**

(54) **CEMENTED CARBIDE BODY CONTAINING ZIRCONIUM AND NIOBIUM AND METHOD OF MAKING THE SAME**

(75) Inventors: **Hans-Wilm Heinrich**, Bayreuth (DE); **Manfred Wolf**, Eckersdorf (DE); **Dieter Schmidt**, Bayreuth (DE)

(73) Assignee: **Kennametal Inc.**, Latrobe, PA (US)

(\*) Notice: Subject to any disclaimer, the term of this patent is extended or adjusted under 35 U.S.C. 154(b) by 97 days.

(21) Appl. No.: **10/727,247**

(22) Filed: **Dec. 3, 2003**

(65) **Prior Publication Data**

US 2005/0120825 A1 Jun. 9, 2005

(51) **Int. Cl.**  
**B22F 3/15** (2006.01)

(52) **U.S. Cl.** ..... **419/13; 419/14; 419/15;**  
**419/18; 419/38; 419/40; 419/60**

(58) **Field of Classification Search** ..... **419/13-15,**  
**419/38, 49, 60, 18**

See application file for complete search history.

(56) **References Cited**

U.S. PATENT DOCUMENTS

- |               |         |                  |       |        |
|---------------|---------|------------------|-------|--------|
| 2,113,355 A * | 4/1938  | McKenna          | ..... | 75/241 |
| 2,731,710 A * | 1/1956  | Lucas et al.     | ..... | 75/242 |
| 3,999,954 A   | 12/1976 | Kolaska et al.   |       |        |
| 4,145,213 A   | 3/1979  | Oskarsson et al. |       |        |
| 4,451,292 A * | 5/1984  | Hall et al.      | ..... | 75/238 |
| 4,843,039 A   | 6/1989  | Akesson et al.   |       |        |
| RE34,180 E    | 2/1993  | Nemeth et al.    |       |        |
| 5,447,549 A   | 9/1995  | Yoshimura        |       |        |
| 5,503,925 A   | 4/1996  | Nakano et al.    |       |        |
| RE35,538 E    | 6/1997  | Akesson et al.   |       |        |
| 5,643,658 A   | 7/1997  | Uchino et al.    |       |        |
| 5,746,803 A   | 5/1998  | Dunmead et al.   |       |        |
| 6,024,776 A   | 2/2000  | Heinrich et al.  |       |        |

6,207,262 B1 \* 3/2001 Ichikawa et al. .... 428/216  
2001/0006594 A1 7/2001 Shibata  
2003/0010166 A1 1/2003 Shibata  
2003/0129456 A1 7/2003 Usami et al.

FOREIGN PATENT DOCUMENTS

|    |              |         |        |
|----|--------------|---------|--------|
| CN | 1425787      | *       | 6/2003 |
| EP | 0 360 567 B1 | 7/1997  |        |
| EP | 0 900 860 A2 | 3/1999  |        |
| EP | 0 900 860 A3 | 11/2002 |        |
| EP | 0 900 860 B1 | 4/2004  |        |
| JP | 02185941 A   | 7/1990  |        |
| JP | 10237650 A   | 9/1998  |        |
| JP | 2002356734 A | 12/2002 |        |
| RU | 2007491      | *       | 2/1994 |

OTHER PUBLICATIONS

PCT Search Report for International Application No. PCT/EP2004/011170 dated Apr. 11, 2005, 12 pages.

\* cited by examiner

Primary Examiner—Ngoclan T. Mai

(74) Attorney, Agent, or Firm—John J. Prizzi

(57) **ABSTRACT**

A sintered cemented carbide body (e.g., a cutting tool) and a method of making the same. The sintered cemented carbide body includes tungsten carbide, a binder phase of at least one metal of the iron group or an alloy thereof, and one or more solid solution phases. Each one of the solid solution phases has at least one of the carbides and carbonitrides of a combination of zirconium, niobium, and tungsten. The method includes the steps of providing a powder mixture that contains tungsten carbide, a binder metal powder comprising at least one metal of the iron group or an alloy thereof, and at least one of the carbides and carbonitrides of both zirconium and niobium including a powder of the carbides or carbonitrides of zirconium and niobium, forming a green compact of said powder mixture, and vacuum sintering or sinter-HIP said green compact at a temperature of from 1400 to 1560° C.

**12 Claims, 4 Drawing Sheets**



FIG. 1



*Fig. 2A*



*Fig. 2B*



*Fig. 3A*



*Fig. 3B*



*Fig. 4*



*Fig. 5*

**CEMENTED CARBIDE BODY CONTAINING  
ZIRCONIUM AND NIOBNIUM AND METHOD  
OF MAKING THE SAME**

BACKGROUND OF THE INVENTION

The present invention provides sintered cemented carbide bodies having increased resistance to plastic deformation comprising tungsten carbide (WC), a binder metal phase and one or more solid solution phases comprising at least one of the carbides, nitrides and carbonitrides of at least one of the elements of groups IVb, Vb and VIb of the Periodic Table of Elements. The present invention also provides a method for producing these sintered cemented carbide bodies. These sintered cemented carbide bodies are useful in the manufacture of cutting tools, and especially indexable cutting inserts for the machining of steel and other metals or metal alloys.

Sintered cemented carbide bodies and powder metallurgical methods for the manufacture thereof are known, for example, from U.S. Pat. Re. 34,180 to Nemeth et al. While cobalt has originally been used as a binder metal for the main constituent, tungsten carbide, a cobalt-nickel-iron alloy as taught by U.S. Pat. No. 6,024,776 turned out to be especially useful as a binder phase for tungsten carbide and other carbides, nitrides and carbonitrides of at least one of the elements titanium, zirconium, hafnium, vanadium, niobium, tantalum, chromium, molybdenum and tungsten, respectively.

Numerous attempts have been made in order to modify the properties or characteristics of the sintered cemented carbide bodies prepared by powder metallurgical methods. These properties include, but are not limited to, hardness, wear resistance, plastic deformation at increased temperatures, density, magnetic properties, resistance to flank wear and resistance to cratering. In order to provide cutting tools having improved wear properties at high cutting speeds, it is known, for example, that the sintered cemented carbide bodies should have increased contents of titanium or tantalum and niobium. On the other hand, however, it is known that increasing contents of titanium or tantalum or niobium result in a noticeable reduction of strength as they form solid solution carbides with tungsten carbide, since the amount of tungsten carbide-phase which provides for the maximum strength in a sintered cemented carbide body decreases with the formation of solid solution carbides.

Also well known to those skilled in the art is the fact that the addition of zirconium and hafnium increases the strength of sintered cemented carbide bodies both at room temperature and at higher temperatures. However, the increase in strength is combined with lower hardness and decreased wear resistance. In addition, a disadvantage of the addition of zirconium is its high affinity to oxygen and its poor wettability which impedes the sintering process used in the preparation of the sintered cemented carbide body.

U.S. Pat. Nos. 5,643,658 and 5,503,925, both hereby incorporated by reference herein, aim at improving hot hardness and wear resistance at higher temperatures of sintered cemented carbide bodies by means of adding zirconium and/or hafnium carbides, nitrides and carbonitrides to the powder mixture of tungsten carbide and a binder metal of the iron family. As a result thereof, the hard phases of at least one of zirconium and hafnium coexist with other hard phases of metals of groups IVb, Vb and VIb, but excluding zirconium and hafnium, with said hard phases forming, in each case, solid solutions with tungsten carbide. Due to the high affinity of zirconium for oxygen, either the starting

powder materials have to be extremely low in oxygen, or the oxygen content has to be controlled by using a reducing sintering atmosphere.

JP-A2-2002-356734, published on Dec. 13, 2002, discloses a sintered cemented carbide body comprising WC, a binder phase consisting of at least one metal of the iron group, and one or more solid solution phases, wherein one of said solid solution phases comprises Zr and Nb while all solid solution phases other than the first one comprise at least one of the elements Ti, V, Cr, Mo, Ta and W, but must not comprise Zr and Nb. According to this Japanese patent document, the best cutting results are achieved at a tantalum content of less than 1% by weight of the total composition, calculated as TaC.

The present invention aims at achieving new sintered cemented carbide bodies having increased resistance to plastic deformation at increased temperatures and, as a result thereof, having increased wear resistance. Besides, the present invention aims at providing a powder metallurgical method of producing said sintered cemented carbide bodies. More specifically, it is an object of the present invention to provide a sintered cemented carbide body having at least two co-existing solid solution phases containing zirconium and niobium or one single homogenous solid solution phase containing zirconium and niobium.

Another object of the present invention consists in providing a method of producing said sintered cemented carbide body comprising the step of providing a powder mixture which upon sintering provides at least two co-existing solid solution phases or one single homogenous solid solution phase containing, in each case, zirconium and niobium, and providing improved sintering activity and wettability with hard constituents of elements of groups IVb, Vb, and VIb of the periodic table of elements.

SUMMARY OF THE INVENTION

In one form thereof, the invention is a sintered cemented carbide body that has increased resistance to plastic deformation. The sintered cemented carbide body includes tungsten carbide, and a binder phase that includes at least one metal of the iron group or an alloy thereof, and one or more solid solution phases wherein each one of the solid solution phases comprises at least one of the carbides and carbonitrides of a combination comprising zirconium, niobium, and tungsten.

In another form thereof, the invention is a method of producing a sintered cemented carbide body comprising the steps of: providing a powder mixture comprising tungsten carbide, a binder metal powder comprising at least one metal of the iron group or an alloy thereof, and at least one of the carbides and carbonitrides of both zirconium and niobium; forming a green compact of said powder mixture; and vacuum sintering or sinter-HIP said green compact at a temperature of from 1400 to 1560° C.

In yet another form thereof, the invention is a cutting tool that comprises a body that includes a rake face and a flank face wherein the rake face and the flank face intersect to form a cutting edge at the intersection thereof. The body comprises tungsten carbide, a binder phase comprising at

least one metal of the iron group or an alloy thereof, and one or more solid solution phases each one of which comprising at least one of the carbides and carbonitrides of a combination comprising zirconium, niobium, and tungsten.

In still another form thereof, the invention is a sintered cemented carbide body that has increased resistance to plastic deformation. The sintered cemented carbide body includes tungsten carbide, and a binder phase that includes at least one metal of the iron group or an alloy thereof, and one or more solid solution phases wherein each one of the solid solution phases comprises at least one of the carbides and carbonitrides of a combination consisting of zirconium, niobium, and tungsten.

#### BRIEF DESCRIPTION OF THE DRAWINGS

The following is a brief description of the drawings that form a part of this patent application:

FIG. 1 is an isometric view of a cutting tool of the present invention wherein the cutting tool is a CNMG style of cutting tool;

FIGS. 2A is a photomicrograph that shows the unetched microstructure of Sample (A), which is a sintered cemented carbide body, at 1,500-fold magnification (10 micrometer scale) wherein Sample (A) was produced according to the present invention as disclosed hereinafter, and Sample (A) has a porosity of <A02 as shown in FIG. 2A;

FIG. 2B is a photomicrograph that shows the unetched microstructures of Sample (B), which is a sintered cemented carbide body, at 1,500-fold magnification (10 micrometer scale) wherein Sample (B) was produced according to a conventional process as disclosed hereinafter, and Sample (B) has a residual porosity of A08 as shown in FIG. 2B;

FIG. 3A is a photomicrograph of a sintered bending strength test rod, in cross section, of Sample (A) which was made according to the present invention as described hereinafter, does not show sinter distortion;

FIG. 3B is a photomicrograph of a sintered bending strength test rod, in cross section, of Sample (B) which was made in a conventional fashion as described hereinafter, very clearly shows a sinter distortion;

FIG. 4 is a photomicrograph (20 micrometer scale) showing the unetched microstructure of an embodiment of the sintered cemented carbide body of the present invention wherein there is shown a binder enriched surface zone free of solid solution carbide wherein the binder enriched surface zone begins at and extends inwardly from the surface of the substrate and one single homogeneous solid solution phase (MC); and

FIG. 5 is a photomicrograph (20 micrometer scale) showing the unetched microstructure of an other embodiment of the sintered cemented carbide body of the present invention wherein there is shown a binder enriched surface zone free of solid solution carbide wherein the binder enriched surface zone begins at and extends inwardly from the surface of the substrate and underneath the binder enriched surface zone free of solid solution phase there is shown a zone in which a single phase MC1 exists (MC1 is light brown), and underneath the MC1 zone there is a zone that has two coexisting solid solution carbide phases wherein one solid solution phase is MC land it is light brown and the other solid solution phase is MC 2 and it is dark brown.

#### DETAILED DESCRIPTION OF SPECIFIC EMBODIMENTS

Referring to FIG. 1, there is shown a cutting tool, i.e., a sintered cemented carbide body, generally designated as 20. Cutting tool 20 has a rake face 22 and flank faces 24. There is a cutting edge 26 at the intersection of the rake face 22 and the flank faces 24. The cutting tool 20 further contains an aperture 28 by which the cutting tool 20 is secured to a tool holder. The style of cutting tool shown in FIG. 5 is a CNMG style of cutting tool. The illustration in FIG. 1 of a CNMG style of cutting tool should not be considered to limit the scope of the invention. It should be appreciated that the present invention is a new cemented carbide material that can be used as a cutting tool wherein the geometry of the cutting tool can be any known cutting tool geometry.

In regard to the composition of the cutting tool, i.e., a sintered cemented carbide body, the composition contains tungsten carbide and a binder, as well as one or more solid solution phases that comprise the carbides and/or the carbonitrides of a combination of zirconium, niobium and tungsten as exemplified by the formulae  $(Zr, Nb, W)C$  and/or  $(Zr, Nb, W)CN$ . In one preferred embodiment of the composition, just one of the solid solution phases consists of a carbide or carbonitride of a combination of zirconium, niobium and tungsten. In another preferred embodiment of the composition, the solid solution phase consisting of a carbide or carbonitride of a combination of zirconium, niobium and tungsten is the sole solid solution phase of the body wherein no other element such as titanium, hafnium, vanadium, tantalum, chromium, and molybdenum is present in said solid solution phase.

In yet another preferred embodiment of the composition, one of the solid solution phases comprises a carbide or carbonitride of a combination of zirconium, niobium and tungsten and at least one carbide, nitride or carbonitride of one or more of titanium, hafnium, vanadium, tantalum, chromium, and molybdenum wherein the solid solution phase may be either the sole solid solution phase of the body or one of two or more different solid solution phases. More specifically, there can be two or more different solid solution phases that are present with each solid solution phase comprising a carbide or carbonitride of a combination of zirconium, niobium and tungsten, and at least one carbide, nitride or carbonitride of one or more of titanium, hafnium, vanadium, tantalum, chromium and molybdenum, respectively. In those cases where the solid solution phase comprises a carbide or carbonitride of a combination of zirconium, niobium and tungsten, and at least one carbide, nitride or carbonitride comprising one or more other metals, it is even more preferred that said at least one other metal is one or more of titanium, tantalum and hafnium.

According to the present invention, the binder alloy preferably comprises cobalt, a CoNi-alloy or a CoNiFe-alloy, each of which may or may not contain additional alloying elements such as chromium and tungsten. The binder alloy preferably comprises between about 3 weight percent to about 15 weight percent of the total body.

Preferably, the total contents of a carbide or carbonitride of a combination of zirconium, niobium and tungsten of the one or more solid solution phase(s) comprise between about 1 weight percent and about 15 weight percent of the total body. Also preferred are those embodiments of the present invention wherein the total content of the elements titanium, hafnium, vanadium, tantalum, chromium and molybdenum does not exceed about 8 weight percent of the total body.

According to especially preferred embodiments of the present invention, titanium comprises between about 1 weight percent and about 8 weight percent of the total body, tantalum comprises between about 1 weight percent and about 7 weight percent of the total body, and hafnium comprises between about 1 weight percent and about 4 weight percent of the total body.

If the cemented carbide body has a mass ratio  $\text{Nb}/(\text{Zr}+\text{Nb})$  of greater than about 0.5, and more preferably greater than or equal to about 0.6, the formation of a single homogeneous solid solution phase or the formation of two or more coexisting solid solution phases within the sintered cemented carbide body is remarkably increased.

According to still another aspect of the present invention, the sintered cemented carbide body comprises at least one of said nitrides or carbonitrides and comprises an outermost zone being free of any solid solution phase but binder enriched up to a depth of about 50 micrometers ( $\mu\text{m}$ ) from an uncoated surface of said body. Embodiments of this type are shown in FIGS. 4 and 5 hereof.

As is acknowledged by those having ordinary skill in the art, binder enrichment and formation of a surface zone free of solid solution carbide (SSC) is induced during sintering once at least one nitride or carbonitride is present in the starting powder mixture. Due to the formation of free nitrogen during sintering, diffusion of binder metal from the bulk towards the surface, and diffusion of solid solution phase from the surface zone towards the bulk will take place, resulting in a binder enriched surface zone being free of any solid solution phase. Due to these diffusion processes, two or more coexisting different solid solution phases showing a concentration gradient between the surface and the center of the body are formed underneath of the binder enriched zone, according to a still more preferred embodiment of the present invention. In those cases, however, where just one single solution phase being homogeneous throughout the body is present, said one single and homogeneous solid solution phase will be located underneath of the binder enriched zone such that the single solid solution phase is homogeneous throughout said body, except in the binder enriched zone.

According to still other preferred embodiments of the present invention, one or more wear resistant layers deposited according to well-known physical vapor deposition (PVD) or chemical vapor deposition (CVD) methods are coated over a surface of the sintered cemented carbide body. Preferably, these wear resistant coatings comprise one or more of the carbides, nitrides, carbonitrides, oxides or borides of a metal of the groups IVb, Vb and VIb of the periodic table of elements, and alumina.

Referring to the method aspects of the present invention, according to a preferred embodiment of the method of the present invention, a solid solution of a carbide or carbonitride of a combination of zirconium and niobium having a mass ratio  $\text{Nb}/(\text{Zr}+\text{Nb})$  of greater than about 0.5, and preferably greater than or equal to about 0.6 or more, is used as the powdered solid solution of a carbide or carbonitride of a combination of zirconium and niobium. The powdered solid solution of a carbide or carbonitride of a combination of zirconium, niobium and tungsten preferably comprises between about 1 weight percent and about 15 weight percent of the total powder mixture.

Preferably, cobalt powder, powders of cobalt and nickel or powders of cobalt and nickel and iron or powders of a cobalt-nickel alloy or powders of a cobalt-nickel-iron alloy are used as the binder metal powders, within the method of the present invention. Optionally, the binder metal powders

may include additional elements, preferably one or more of chromium and tungsten. Preferably, the binder metal powder comprises between about 3 weight percent and about 15 weight percent of the total powder mixture.

According to still another embodiment of the present invention, the powder mixture additionally comprises at least one carbide, nitride or carbonitride of one or more of titanium, hafnium, vanadium, tantalum, chromium, and molybdenum. Preferably, the powder mixture comprises at least one of the elements titanium, hafnium, vanadium, tantalum, chromium and molybdenum in an amount of between about 1 weight percent and about 8 weight percent of the total powder mixture.

The present inventors have surprisingly found that due to the addition of zirconium and niobium in the form of a powdered solid solution of a carbide or carbonitride of a combination of zirconium and niobium to the starting powder mixture, instead of using zirconium carbide plus niobium carbide or zirconium carbonitride plus niobium carbonitride, each individually, either one single homogeneous solid solution phase comprising the carbides and/or the carbonitrides of a combination of zirconium, niobium and tungsten, or two or more coexisting solid solution phases comprising the carbides and/or the carbonitrides of a combination of zirconium, niobium and tungsten, and at least one carbide, nitride or carbonitride of one or more of titanium, hafnium, vanadium, tantalum, chromium and molybdenum, depending on the compounds added to the starting powder mixture, are formed during sintering according to the method of the present invention.

Contrary to the documents mentioned herein above, upon sintering all elements added to the starting powder mixture are dissolved in each one of the coexisting solid solution phases, according to the present invention. For example, up to about 65 weight percent tungsten, up to about 75 weight percent niobium, up to about 60 weight percent zirconium, up to about 20 weight percent titanium, up to about 15 weight percent tantalum, and up to about 20 weight percent hafnium can be dissolved in the coexisting solid solution phases.

Another advantage of the use of a powdered solid solution of a carbide or carbonitride of a combination of zirconium and niobium as part of the starting powder mixture according to the present invention is the fact that tantalum can be added to the composition for improving binder phase distribution and toughness in an amount of about 1 weight percent or more of the total starting powder mixture.

The best results in terms of homogeneity of the solid solution phase(s) formed according to the present invention have been obtained if a powdered solid solution of a carbide or carbonitride of a combination of zirconium and niobium having a ratio of about 40 weight percent zirconium carbide and about 60 weight percent niobium carbide was added to the starting powder mixture.

Referring to FIG. 2A and FIG. 2B, each one of these figures is a photomicrograph at 1500 $\times$ (each photomicrograph as a 10 micrometer scale) that shows the unetched microstructures of two samples; namely, Sample (A) and Sample (B), respectively. Sample (A) was produced according to the present invention using  $(\text{Zr},\text{Nb})\text{C}$  in the starting powder mixture and whereas Sample (B) was conventionally made by using individual carbides; namely,  $\text{ZrC}$  and  $\text{NbC}$  instead of  $(\text{Zr},\text{Nb})\text{C}$  in the starting powder mixture. FIG. 2A shows that Sample (A) has a porosity of less than A02 and FIG. 2B shows that Sample (B) has a porosity of A08. In addition, as can be seen in FIG. 2A, the microstructure of Sample (A) obtained by using the  $(\text{Zr},\text{Nb})\text{C}$  solid

solution in the starting powder is much more homogeneous in terms of porosity as compared with the microstructure (see FIG. 2B) of Sample (B), which is the conventionally prepared sintered cemented carbide body using ZrC+NbC as part of the starting powder mixture.

Referring to FIG. 3A and FIG. 3B, these figures are photomicrographs of sintered bending strength test rods wherein each is in cross section. FIG. 3B shows the microstructure of Sample (B) that is made in a conventional fashion using ZrC and NbC in the starting powder mixture wherein there is a sinter distortion that can be seen very clearly. FIG. 3A shows the microstructure of Sample (A) that was made according to the present invention using a solid solution carbide of zirconium and niobium (Zr,Nb)C wherein FIG. 3A does not show sinter distortion. This comparison shows that with respect to sinter distortion, Sample (A) is much better than the conventional Sample (B).

As indicated earlier, a further advantage of using a powdered solid solution of a carbide or carbonitride of a combination of zirconium and niobium as part of the starting powder mixture consists in the lower affinity to oxygen, as compared to conventional methods of producing sintered cemented carbide bodies, whereby it is not necessary to have a reducing sintering atmosphere. Due to the avoidance of any controlling and monitoring of the reducing quality of the sintering atmosphere, sintering becomes easier and less expensive according to the present invention as compared to the prior art.

Referring to FIG. 4, FIG. 4 is a photomicrograph of an embodiment of the sintered cemented carbide body of the present invention wherein there is shown a binder enriched surface zone free of solid solution carbide and one single homogeneous solid solution phase (MC). FIG. 4 shows that the present invention allows the production of sintered cemented carbide bodies having one single homogeneous solid solution phase as shown.

Referring to FIG. 5, FIG. 5 is a photomicrograph of an other embodiment of the sintered cemented carbide body of the present invention wherein there is shown a binder enriched surface zone free of solid solution carbide. Underneath the binder enriched surface zone free of solid solution phase there is shown a zone in which a solid solution phase MC1 exists. MC1 is light brown. Underneath the zone containing only MC1 solid solution phase, there is a zone that contains two coexisting solid solution phases. One solid solution phase is MC1 and it is light brown. The other solid solution phase is MC2 and it is dark brown. FIG. 5 shows that the present invention allows the production of sintered cemented carbide bodies having different coexisting solid solution phases (MC1; (MC1+MC2)) visible by optical microscopy located underneath an outermost binder enriched zone being free of solid solution phase.

Further details of the invention shall be described through the following examples. Table 1 sets forth the raw materials that were used in the examples that are set forth hereinafter.

TABLE 1

| Raw Materials Used for the Examples |              |                                         |
|-------------------------------------|--------------|-----------------------------------------|
| Raw material                        | Manufacturer | Average particle size [ $\mu\text{m}$ ] |
| Co                                  | OMG          | 1.3                                     |
| (W, Ti)C 50/50                      | H.C. Starck  | 1.1                                     |
| NbC                                 | Kennametal   | 1.5                                     |
| TaC                                 | Kennametal   | 1.2                                     |

TABLE 1-continued

| Raw Materials Used for the Examples |              |                                         |
|-------------------------------------|--------------|-----------------------------------------|
| Raw material                        | Manufacturer | Average particle size [ $\mu\text{m}$ ] |
| (Ta, Nb)C 70/30                     | H.C. Starck  | 2.1                                     |
| HfC                                 | Cezus        | 0.5                                     |
| ZrC                                 | H.C. Starck  | 3.0                                     |
| (Zr, Nb)C 40/60                     | H.C. Starck  | 1.7                                     |
| (Zr, Nb)C 50/50                     | H.C. Starck  | 1.1                                     |
| TiC/N 70/30                         | H.C. Starck  | 1.5                                     |
| TiN                                 | H.C. Starck  | 1.1                                     |
| WC 1                                | Kennametal   | 1.0                                     |
| WC 2                                | Kennametal   | 2.5                                     |
| WC 3                                | Kennametal   | 8.0                                     |
| WC 4                                | Kennametal   | 12.0                                    |

In regard to the processing of the examples, for each one of the examples the specified raw materials were wet milled in an attritor for 10 hours and dried. Green compacts were pressed of the resulting powder mixtures and sintered according to the sintering conditions stated in the examples. In the examples the percentages are given in weight percent unless otherwise stated.

As is well known to those skilled in the art of powder metallurgy, the element pairs tantalum and niobium as well as zirconium and hafnium in most cases of occurrence are associated with each other such that a complete separation often is difficult to obtain. This is why in commercial applications, small amounts or traces of niobium will be present in tantalum, and vice versa, and small amounts or traces of zirconium will be present in hafnium, and vice versa. This also is valid for the present disclosure, whenever these elements or compounds thereof are mentioned by their names or chemical formulae.

## EXAMPLE 1

Powder mixtures A and B having the compositions (weight percent) given in Table 2 were prepared. TRS bars (ISO 3327, type B) were pressed from these powder mixtures to form green compacts. The compacts were sintered-HIPped at temperatures between 1430 and 1520 degrees Centigrade. The resulting sintered cemented carbide bodies were metallurgically tested. The results of these tests are shown in FIGS. 2A and 2B and FIGS. 3A and 3B. Sample A (according to the present invention) shows a porosity of <A02 (see FIG. 2A), whereas sample B (prior art comparative example) shows a high residual porosity (see FIG. 2B) and strong sinter distortion (see FIG. 3B).

TABLE 2

| Starting Powder Mixtures for Samples (A) and (B) (weight percent) |    |                 |     |     |         |
|-------------------------------------------------------------------|----|-----------------|-----|-----|---------|
| Sample                                                            | Co | (Zr, Nb)C 50/50 | ZrC | NbC | WC2     |
| (A)                                                               | 10 | 15              |     |     | balance |
| (B)                                                               | 10 |                 | 7.5 | 7.5 | balance |

The resulting sintered cemented carbide bodies of Sample (A) and Sample (B) had the following properties as reported in Table 3 below.

TABLE 3

| Selected Properties for Sample (A) and Sample (B) |                                 |                                                      |         |                  |                                       |
|---------------------------------------------------|---------------------------------|------------------------------------------------------|---------|------------------|---------------------------------------|
|                                                   | Density<br>[g/cm <sup>3</sup> ] | Magnetic<br>Saturation<br>[0.1 μTm <sup>3</sup> /kg] | Hc [Oe] | Hardness<br>HV30 | Porosity/<br>Remarks                  |
| A                                                 | 12.58                           | 182                                                  | 167     | 1500             | <A02, OK<br>(no sinter<br>distortion) |
| B                                                 | 12.51                           | 188                                                  | 155     | 1500             | A08,<br>sinter<br>distortion          |

In regard to the columns of Table 3, the density is reported in grams per cubic centimeter, the magnetic saturation is reported in 0.1 micro tesla cubic meter per kilogram, the coercive force (H<sub>C</sub>) is reported in oersteds, the hardness is reported as a Vickers Hardness Number using a 30 kilogram load, and the porosity was ascertained per a visual inspection. The test methods used to determine the properties set forth in Table 3, as well as throughout the entire patent application, are described below. The method to determine density was according to ASTM Standard B311-93(2002)e1 entitled "Test Method for Density Determination for Powder Metallurgy (P/M) Materials Containing Less Than Two Percent Porosity. The method used to determine the magnetic saturation was along the lines of ASTM Standard B886-03 entitled "Standard Test Methods for Determination of MAGNETIC Saturation (Ms) of Cemented Carbides. The method to determine coercive force was ASTM Standard B887-03 entitled "Standard Test Method for Determination of Coercivity (Hcs) for Cemented Carbides. The method to determine the Vickers hardness was along the lines of ASTM Standard E92-82(2003)e1 entitled "Standard Test Method for VICKERS Hardness of Metallic Materials". The method used to determine the porosity was along the lines of ASTM Standard B276-91(2000) entitled "Standard Test Method for Apparent Porosity in Cemented Carbides".

## EXAMPLE 2

Similar to Example 1, powder mixtures C through G were prepared, as given in Table 4 below.

TABLE 4

| Starting Powder Mixtures for Samples C through G |                    |                  |     |      |         |
|--------------------------------------------------|--------------------|------------------|-----|------|---------|
|                                                  | (Zr, Nb)C<br>50/50 | TiC <sup>†</sup> | TaC | HfC  | WC3     |
| C                                                | 6.0                | 7.5              |     |      | balance |
| D                                                | 6.0                | 5.0              | 2.5 |      | balance |
| E                                                | 6.0                | 3.25             | 2.5 | 1.75 | balance |
| F                                                | 6.0                | 3.0              | 2.5 | 1.0  | balance |
| G                                                | 6.0                | 2.5              | 2.5 | 5.0* | balance |

\*as (Ta, Nb)C 70/30

<sup>†</sup>as (W, Ti)C 50/50

Cutting inserts were pressed from powder mixtures C to G in geometry CNMG120412-UN, then sintered (sinter-HIP 1505° C/85 min) and CVD coated to form a standard multilayer coating comprised of titanium carbonitride and

alumina layers. All samples were coated equally. The resulting sintered bodies had the following properties as set forth in Table 5 below.

TABLE 5

| Selected Properties for Samples C through G |                                 |                                                      |            |                  |
|---------------------------------------------|---------------------------------|------------------------------------------------------|------------|------------------|
|                                             | Density<br>[g/cm <sup>3</sup> ] | Magnetic<br>Saturation<br>[0.1 μTm <sup>3</sup> /kg] | Hc<br>[Oe] | Hardness<br>HV30 |
| 10                                          |                                 |                                                      |            |                  |
| 15                                          | C                               | 13.95                                                | 91         | 199              |
|                                             | D                               | 13.56                                                | 106        | 216              |
|                                             | E                               | 13.72                                                | 106        | 189              |
|                                             | F                               | 13.66                                                | 108        | 185              |
| 20                                          | G                               | 13.88                                                | 111        | 165              |

These cutting inserts were subjected to deformation resistance turning tests under the following conditions:

25 Workpiece material: 42 CrMo4 (1.7225)—alloy steel  
Cutting speed: 500, 550 m/min, from 550 m/min in stages  
of 25 m/min increasing up to failure of the insert due to  
plastic deformation because of thermal overloading.  
30 Cutting time: 15 sec. for each cutting speed  
Feed rate: 0.4 mm/rev.  
Cutting depth: 2.5 mm  
Coolant: none

The results of these tests are set forth in Table 6 below.

TABLE 6

| Test Results for Examples C through G |                   |                                          |             |    |             |             |
|---------------------------------------|-------------------|------------------------------------------|-------------|----|-------------|-------------|
| Cutting<br>speed<br>m/min             | G<br>Prior art    | Cutting time per cutting speed [seconds] |             |    |             |             |
|                                       |                   | C                                        | D           | E  | F           |             |
| 45                                    | 500               | 15                                       | 15          | 15 | 15          | 15          |
|                                       | 550               | 15                                       | 15          | 15 | 15          | 15          |
|                                       | 575               | not reached                              | 15          | 15 | 15          | 15          |
|                                       | 600               | not reached                              | 15          | 15 | 15          | 15          |
| 50                                    | 625               | not reached                              | 4           | 15 | 8           | 13          |
|                                       | 650               | not reached                              | not reached | 2  | not reached | not reached |
| 55                                    | Σ cutting<br>time | 30                                       | 64          | 77 | 68          | 73          |

Further, CVD coated (same coatings as in Example 2) cutting inserts from powder mixtures C to G were subjected to a wear turning test under the following parameters:

60 Workpiece material: 42 CrMo4 (1.7225)-alloy steel  
Cutting speed: 320 and 340 m/min  
Cutting time: 2 min for each cutting speed  
Feed rate: 0.3 mm/rev.  
Cutting depth: 2.5 mm  
Coolant: none

The results are set forth in Table 7 below that report the amount of flank wear in millimeters.

TABLE 7

| Results of Testing of Samples C through G |                 |      |      |      |      |  |
|-------------------------------------------|-----------------|------|------|------|------|--|
| Cutting speed                             | Flank wear [mm] |      |      |      |      |  |
| m/min                                     | G Prior art     | C    | D    | E    | F    |  |
| 320                                       | 0.19            | 0.17 | 0.15 | 0.19 | 0.17 |  |
| 340                                       | 0.70            | 0.30 | 0.19 | 0.33 | 0.24 |  |

Test pieces were pressed and sintered with powder mixtures D, C, F and G. These test pieces were subjected to a hot hardness test (Vickers hardness) under the following conditions:

Test weight: 1000 grams

Test temperatures: room temperature RT, 400, 600, 800 and 900° C.

The results of the hardness testing are set forth in Table 8 below.

TABLE 8

| Results of Vickers Hardness Testing for Samples D, C, F and G |      |         |         |         |         |
|---------------------------------------------------------------|------|---------|---------|---------|---------|
| Sample                                                        | RT   | 400° C. | 600° C. | 800° C. | 900° C. |
| D                                                             | 1685 | 1460    | 1180    | 789     | 599     |
| C                                                             | 1686 | 1372    | 1062    | 718     | 536     |
| F                                                             | 1710 | 1375    | 1116    | 730     | 553     |
| G prior art                                                   | 1636 | 1174    | 969     | 645     | 498     |

Just as with the hot hardness turning tests, the Vickers hardness (hot hardness) test shows for the sintered bodies according to the present invention a clearly increased resistance against plastic deformation at higher temperatures as compared to the prior art.

The compositions of the solid solution carbide (SSC) phase of samples C, D, E and F were analyzed by scanning electron microscopy (SEM) with the assistance of EDAX. In samples D, E and F two different SSC-phases could be identified by optical microscopy, whereas sample C showed one single SSC-phase, only. Where two different SSC-phases were present, the darker one was richer in tungsten and lower in zirconium, as compared with the lighter one. The results of the above determination are reported in Table 9 below that presents the composition of the solid solution carbides (as sintered) in weight percent.

TABLE 9

| Compositions of Solid Solution Phases for Samples C, D, E and F |       |       |       |       |      |       |                                        |
|-----------------------------------------------------------------|-------|-------|-------|-------|------|-------|----------------------------------------|
|                                                                 | Zr    | Nb    | Ti    | W     | Ta   | Hf    | SSC-phases found by optical microscopy |
| C                                                               | 25-40 | 40-75 |       | 1-25  |      |       | 1                                      |
| D                                                               | 12-15 | 18-28 | 9-15  | 45-65 |      |       | 2                                      |
|                                                                 | 40-52 | 23-45 | 1-6   | 4-27  |      |       |                                        |
| E                                                               | 7-10  | 10-17 | 12-17 | 48-62 | 5-13 |       | 2                                      |
|                                                                 | 43-58 | 15-25 | 3-6   | 12-32 | 5-10 |       |                                        |
| F                                                               | 5-9   | 10-16 | 13-20 | 48-56 | 8-13 | 1-6   | 2                                      |
|                                                                 | 15-43 | 7-19  | 4-11  | 15-43 | 1-10 | 10-19 |                                        |

## EXAMPLE 3

Similar to Example 1, powder mixtures H through K as given in Table 10 were prepared:

TABLE 10

| Starting Powder Mixtures for Samples H through K |     |                 |                  |     |         |
|--------------------------------------------------|-----|-----------------|------------------|-----|---------|
|                                                  | Co  | (Zr, Nb)C 50/50 | TiC <sup>†</sup> | TaC | WC*     |
| H                                                | 6.0 | 2.0             |                  |     | balance |
| I                                                | 6.0 | 2.0             | 0.5              |     | balance |
| J                                                | 6.0 | 2.0             | 1.0              |     | balance |
| K                                                | 6.0 |                 |                  | 3.5 | balance |

\*Mixture of WC1 and WC2: 75% WC1, 25% WC2

<sup>†</sup>as (W, Ti)C 50/50

From powder mixtures H, I, J and K (prior art), cutting inserts having the geometry CNMG120412-UN were manufactured, pressed, sintered/sinter-HIP (1505° C./85 min) and CVD coated. The resulting sintered bodies had the following properties as reported in Table 11.

TABLE 11

| Selected properties of Samples H through K |                              |                                               |         |               |
|--------------------------------------------|------------------------------|-----------------------------------------------|---------|---------------|
|                                            | Density [g/cm <sup>3</sup> ] | Magnetic Saturation [0.1 Tm <sup>3</sup> /kg] | Hc [Oe] | Hardness HV30 |
| H                                          | 14.71                        | 95                                            | 253     | 1660          |
| I                                          | 14.57                        | 96                                            | 300     | 1700          |
| J                                          | 14.42                        | 100                                           | 289     | 1680          |
| K                                          | 14.89                        | 96                                            | 245     | 1640          |

These cutting inserts were subjected to hot hardness tests under the following conditions:

Workpiece material: 42 CrMo4 (1.7225)—alloy steel  
Cutting speed: increasing from 450 m/min in stages of 25 m/min until failure of the inserts due to plastic deformation because of thermal overloading.

Cutting time: 15 sec. for each cutting speed  
Feed rate: 0.4 mm/rev.

Cutting depth: 2.5 µm

Coolant: none

## 13

The results of these cutting tests are set forth in Table 12 below.

TABLE 12

| Cutting speed<br>m/min | Results of Cutting Tests for Samples K through J |             |             |             |
|------------------------|--------------------------------------------------|-------------|-------------|-------------|
|                        | Cutting time per cutting speed [seconds]         |             |             |             |
| speed<br>m/min         | K<br>Prior art                                   | H           | I           | J           |
| 450                    | 15                                               | 15          | 15          | 15          |
| 475                    | 15                                               | 15          | 15          | 15          |
| 500                    | 9                                                | 15          | 15          | 15          |
| 525                    | not reached                                      | 2           | 13          | 15          |
| 550                    | not reached                                      | not reached | not reached | 5           |
| 575                    | not reached                                      | not reached | not reached | not reached |
| $\Sigma$ time          | 39                                               | 47          | 58          | 65          |

A review of these test results show a tool life improvement between about 20 percent and about 67 percent.

Further inserts made from mixtures H to K and CVD coated. These coated inserts were subjected to a wear turning test with increasing cutting speeds under the following parameters:

Workpiece material: 42 CrMo4 (1.7225)—alloy steel

Cutting speed: 260, 300, 320 and 340 m/min

Cutting time: 2 min each cutting speed

Feed rate: 0.5 mm/rev.

Cutting depth: 1.5 mm

Coolant: none

The results are set forth in Table 13.

TABLE 13

| Cutting speed<br>m/min | Results of Cutting Tests for Coated Samples K through J |      |      |      |
|------------------------|---------------------------------------------------------|------|------|------|
|                        | Flank wear [mm]                                         |      |      |      |
| speed<br>m/min         | K<br>Prior art                                          | H    | I    | J    |
| 260                    | 0.14                                                    | 0.14 | 0.13 | 0.13 |
| 300                    | 0.20                                                    | 0.20 | 0.17 | 0.17 |
| 320                    | 0.31                                                    | 0.25 | 0.21 | 0.21 |
| 340                    | not reached                                             | 0.39 | 0.29 | 0.29 |

## EXAMPLE 4

Powder mixtures L and M (prior art) were prepared according to the compositions given in Table 14 (the compositions are set forth in weight percent below):

TABLE 14

| Starting Powder Mixtures for Samples L and M |                    |                  |     |               |      |            |
|----------------------------------------------|--------------------|------------------|-----|---------------|------|------------|
| Co                                           | (Zr, Nb)C<br>50/50 | TiC <sup>†</sup> | TiN | TiCN<br>70/30 | TaC  | NbC<br>WC4 |
| L                                            | 6.3                | 4.0              | 0.8 | 1.2           | 1.0  | 0.3        |
| M                                            | 6.3                |                  | 1.7 | 0.8           | 5.4* | balance    |

\*as (Ta, Nb)C 70/30

<sup>†</sup>as (W, Ti)C 50/50

Cutting inserts were pressed from powder mixtures L and M in geometry CNMG120412-UN, then sintered (sinter-HIP

## 14

1505° C./85 min) and CVD coated. The resulting sintered bodies had the following properties as reported in Table 15. In addition to the properties reported for the above examples, Table 15 also reports the depth of the cobalt-enriched SSC-free zone in micrometers and the volume percent of cubic carbides present except for tungsten carbide.

TABLE 15

| Selected Properties of Cutting Inserts of Samples L and M |                                 |                                                      |            |                  |                                         |                             |
|-----------------------------------------------------------|---------------------------------|------------------------------------------------------|------------|------------------|-----------------------------------------|-----------------------------|
|                                                           | Density<br>[g/cm <sup>3</sup> ] | Magnetic<br>Saturation<br>[0.1 μTm <sup>3</sup> /kg] | Hc<br>[Oe] | Hardness<br>HV30 | Co<br>enriched<br>SSC free<br>zone [μm] | Cubic<br>Carbides<br>Vol.-% |
| L                                                         | 13.57                           | 114                                                  | 166        | 1460             | 25                                      | 14.8                        |
| M                                                         | 13.92                           | 113                                                  | 149        | 1460             | 25                                      | 13.7                        |

These cutting inserts were subjected to a toughness test (interrupted cutting test) with the following conditions:

Workpiece material: Ck60 (1.1221)—carbon steel

Cutting speed: 200 m/min

Cutting depth: 2.5 mm

Feed rate: 0.3, 0.4, 0.5 mm/rev., 100 impacts per feed rate.

Coolant: none

The feed was increased according to the mentioned increments until breakage occurred. Table 16 below sets forth the results of the toughness test.

TABLE 16

| Results of Toughness Test (Interrupted Cutting) for Samples L and M |                               |          |          |         |
|---------------------------------------------------------------------|-------------------------------|----------|----------|---------|
|                                                                     | No. of impacts until breakage |          |          |         |
|                                                                     | Insert 1                      | Insert 2 | Insert 3 | Average |
| L                                                                   | 950                           | 875      | 950      | 925     |
| M prior art                                                         | 875                           | 692      | 820      | 796     |

Additional cutting inserts were subjected to a deformation resistance turning test under following conditions:

Workpiece material: 42 CrMo4 (1.7225)—alloy steel

Cutting speed: 400, 430, 460 m/min in stages of 30 m/min increasing up to failure of the insert due to plastic deformation because of thermal overloading

Cutting time: 5 sec. for each cutting speed

Cutting depth: 2.5 mm

Feed rate: 0.3 mm/rev.

Coolant: none

Table 17 sets for the results of these deformation resistance turning tests.

TABLE 17

| Results of Deformation Resistance Turning Tests for Samples L and M |                |         |
|---------------------------------------------------------------------|----------------|---------|
| Cutting speed<br>m/min                                              | M<br>Prior Art | L       |
| 400                                                                 | 5              | 5       |
| 430                                                                 | 5              | 5       |
| 460                                                                 | not reached    | 5       |
| 490                                                                 | not reached    | 5       |
| Total<br>Cutting Time                                               | 10 sec.        | 20 sec. |

Further cutting inserts were subjected to a wear turning test under the following conditions:

Workpiece material: 42 CrMo4 (1.7225)—alloy steel  
 Cutting speed: 208 m/min  
 Cutting depth: 2.5 mm  
 Feed rate: 0.4 mm/rev.  
 Coolant: none

The results of the wear turning test are reported in Table 18 below.

TABLE 18

| Results of Wear Turning Tests for Samples L and M |                 |       |
|---------------------------------------------------|-----------------|-------|
| Cutting time                                      | Flank wear [mm] |       |
|                                                   | M prior Art     | L     |
| 2 min                                             | 0.191           | 0.153 |
| 4 min                                             | 0.352           | 0.250 |
| (End of Life)                                     |                 |       |

## EXAMPLE 5

Powder mixtures N and O were prepared having the compositions (in weight percent) given in Table 19.

TABLE 19

| Starting Powder Compositions for Samples N and O |           |       |                  |       |     |     |
|--------------------------------------------------|-----------|-------|------------------|-------|-----|-----|
| Co                                               | (Zr, Nb)C |       | TiCN             |       | WC3 |     |
|                                                  | 50/50     | 40/60 | TiC <sup>†</sup> | 70/30 | TaC | NbC |
| N                                                | 6.0       | 8.0   |                  | 1.0   | 1.5 | 0.4 |
| O                                                | 6.0       |       | 10.0             | 1.0   | 1.5 | 0.4 |

<sup>†</sup>as (W, Ti)C 50/50

From starting powder mixtures N and O, green compacts were pressed (TRS bars, ISO 3327, type B) and vacuum sintered at 1530° C./60 min. The as sintered properties of Samples N and O are set forth in Table 20 below:

TABLE 20

| Selected Properties of Samples N and O |                                 |                                                      |                  |                                      |
|----------------------------------------|---------------------------------|------------------------------------------------------|------------------|--------------------------------------|
|                                        | Density<br>[g/cm <sup>3</sup> ] | Magnetic<br>Saturation<br>[0.1 μTm <sup>3</sup> /kg] | Hardness<br>HV30 | Co enriched<br>SSC free<br>zone [μm] |
| N                                      | 13.10                           | 108                                                  | 221              | 1610                                 |
| O                                      | 12.89                           | 103                                                  | 206              | 1660                                 |

An analysis of the sintered bodies revealed that Sample N shows two different coexisting solid solution phases that were identified by optical microscopy. By optical microscopy Sample O showed one single homogeneous solid solution phase. The compositional results of the analysis of Samples N and O are set forth in Table 21 below.

TABLE 21

| Composition of solid solution carbides (as sintered) in Samples N and O<br>(components are set forth in weight percent) |       |       |       |      |       |      |
|-------------------------------------------------------------------------------------------------------------------------|-------|-------|-------|------|-------|------|
|                                                                                                                         |       | Zr    | Nb    | Ti   | W     | Ta   |
| N                                                                                                                       | SSC1* | 12-17 | 19-22 | 8-13 | 44-48 | 8-11 |
|                                                                                                                         | SSC2  | 33-38 | 49-57 | 1-4  | 2-10  | 2-7  |
| O                                                                                                                       |       | 13-16 | 24-28 | 8-10 | 39-45 | 7-10 |

\*Thickness of SSC1-zone: about 80 to 120 μm

15 The problems of the prior art mentioned above are overcome by the present invention which provides a sintered cemented carbide body having increased resistance to plastic deformation, comprising tungsten carbide, a binder phase comprising at least one metal of the iron group or an alloy thereof, and one or more solid solution phases each one of which comprising at least one of the carbides and carbonitrides of a combination of zirconium, niobium, and tungsten. Further, the problems of the prior art are overcome by the method of the present invention wherein this method is a method of producing said sintered cemented carbide body, according to the present invention, comprises the steps of:

- providing a powder mixture comprising tungsten carbide, a binder metal powder comprising at least one metal of the iron group or an alloy thereof, and at least one of the carbides and carbonitrides of both, zirconium and niobium;
- forming a green compact of said powder mixture;
- vacuum sintering or sinter-HIP said green compact at a temperature of from 1400 to 1560° C.;

35 20 25 30 35 40 45 50 55 60 65 70 75 80 85 90 95 100 105 110 115 120 125 130 135 140 145 150 155 160 165 170 175 180 185 190 195 200 205 210 215 220 225 230 235 240 245 250 255 260 265 270 275 280 285 290 295 300 305 310 315 320 325 330 335 340 345 350 355 360 365 370 375 380 385 390 395 400 405 410 415 420 425 430 435 440 445 450 455 460 465 470 475 480 485 490 495 500 505 510 515 520 525 530 535 540 545 550 555 560 565 570 575 580 585 590 595 600 605 610 615 620 625 630 635 640 645 650 655 660 665 670 675 680 685 690 695 700 705 710 715 720 725 730 735 740 745 750 755 760 765 770 775 780 785 790 795 800 805 810 815 820 825 830 835 840 845 850 855 860 865 870 875 880 885 890 895 900 905 910 915 920 925 930 935 940 945 950 955 960 965 970 975 980 985 990 995 1000 1005 1010 1015 1020 1025 1030 1035 1040 1045 1050 1055 1060 1065 1070 1075 1080 1085 1090 1095 1100 1105 1110 1115 1120 1125 1130 1135 1140 1145 1150 1155 1160 1165 1170 1175 1180 1185 1190 1195 1200 1205 1210 1215 1220 1225 1230 1235 1240 1245 1250 1255 1260 1265 1270 1275 1280 1285 1290 1295 1300 1305 1310 1315 1320 1325 1330 1335 1340 1345 1350 1355 1360 1365 1370 1375 1380 1385 1390 1395 1400 1405 1410 1415 1420 1425 1430 1435 1440 1445 1450 1455 1460 1465 1470 1475 1480 1485 1490 1495 1500 1505 1510 1515 1520 1525 1530 1535 1540 1545 1550 1555 1560 1565 1570 1575 1580 1585 1590 1595 1600 1605 1610 1615 1620 1625 1630 1635 1640 1645 1650 1655 1660 1665 1670 1675 1680 1685 1690 1695 1700 1705 1710 1715 1720 1725 1730 1735 1740 1745 1750 1755 1760 1765 1770 1775 1780 1785 1790 1795 1800 1805 1810 1815 1820 1825 1830 1835 1840 1845 1850 1855 1860 1865 1870 1875 1880 1885 1890 1895 1900 1905 1910 1915 1920 1925 1930 1935 1940 1945 1950 1955 1960 1965 1970 1975 1980 1985 1990 1995 2000 2005 2010 2015 2020 2025 2030 2035 2040 2045 2050 2055 2060 2065 2070 2075 2080 2085 2090 2095 2100 2105 2110 2115 2120 2125 2130 2135 2140 2145 2150 2155 2160 2165 2170 2175 2180 2185 2190 2195 2200 2205 2210 2215 2220 2225 2230 2235 2240 2245 2250 2255 2260 2265 2270 2275 2280 2285 2290 2295 2300 2305 2310 2315 2320 2325 2330 2335 2340 2345 2350 2355 2360 2365 2370 2375 2380 2385 2390 2395 2400 2405 2410 2415 2420 2425 2430 2435 2440 2445 2450 2455 2460 2465 2470 2475 2480 2485 2490 2495 2500 2505 2510 2515 2520 2525 2530 2535 2540 2545 2550 2555 2560 2565 2570 2575 2580 2585 2590 2595 2600 2605 2610 2615 2620 2625 2630 2635 2640 2645 2650 2655 2660 2665 2670 2675 2680 2685 2690 2695 2700 2705 2710 2715 2720 2725 2730 2735 2740 2745 2750 2755 2760 2765 2770 2775 2780 2785 2790 2795 2800 2805 2810 2815 2820 2825 2830 2835 2840 2845 2850 2855 2860 2865 2870 2875 2880 2885 2890 2895 2900 2905 2910 2915 2920 2925 2930 2935 2940 2945 2950 2955 2960 2965 2970 2975 2980 2985 2990 2995 3000 3005 3010 3015 3020 3025 3030 3035 3040 3045 3050 3055 3060 3065 3070 3075 3080 3085 3090 3095 3100 3105 3110 3115 3120 3125 3130 3135 3140 3145 3150 3155 3160 3165 3170 3175 3180 3185 3190 3195 3200 3205 3210 3215 3220 3225 3230 3235 3240 3245 3250 3255 3260 3265 3270 3275 3280 3285 3290 3295 3300 3305 3310 3315 3320 3325 3330 3335 3340 3345 3350 3355 3360 3365 3370 3375 3380 3385 3390 3395 3400 3405 3410 3415 3420 3425 3430 3435 3440 3445 3450 3455 3460 3465 3470 3475 3480 3485 3490 3495 3500 3505 3510 3515 3520 3525 3530 3535 3540 3545 3550 3555 3560 3565 3570 3575 3580 3585 3590 3595 3600 3605 3610 3615 3620 3625 3630 3635 3640 3645 3650 3655 3660 3665 3670 3675 3680 3685 3690 3695 3700 3705 3710 3715 3720 3725 3730 3735 3740 3745 3750 3755 3760 3765 3770 3775 3780 3785 3790 3795 3800 3805 3810 3815 3820 3825 3830 3835 3840 3845 3850 3855 3860 3865 3870 3875 3880 3885 3890 3895 3900 3905 3910 3915 3920 3925 3930 3935 3940 3945 3950 3955 3960 3965 3970 3975 3980 3985 3990 3995 4000 4005 4010 4015 4020 4025 4030 4035 4040 4045 4050 4055 4060 4065 4070 4075 4080 4085 4090 4095 4100 4105 4110 4115 4120 4125 4130 4135 4140 4145 4150 4155 4160 4165 4170 4175 4180 4185 4190 4195 4200 4205 4210 4215 4220 4225 4230 4235 4240 4245 4250 4255 4260 4265 4270 4275 4280 4285 4290 4295 4300 4305 4310 4315 4320 4325 4330 4335 4340 4345 4350 4355 4360 4365 4370 4375 4380 4385 4390 4395 4400 4405 4410 4415 4420 4425 4430 4435 4440 4445 4450 4455 4460 4465 4470 4475 4480 4485 4490 4495 4500 4505 4510 4515 4520 4525 4530 4535 4540 4545 4550 4555 4560 4565 4570 4575 4580 4585 4590 4595 4600 4605 4610 4615 4620 4625 4630 4635 4640 4645 4650 4655 4660 4665 4670 4675 4680 4685 4690 4695 4700 4705 4710 4715 4720 4725 4730 4735 4740 4745 4750 4755 4760 4765 4770 4775 4780 4785 4790 4795 4800 4805 4810 4815 4820 4825 4830 4835 4840 4845 4850 4855 4860 4865 4870 4875 4880 4885 4890 4895 4900 4905 4910 4915 4920 4925 4930 4935 4940 4945 4950 4955 4960 4965 4970 4975 4980 4985 4990 4995 5000 5005 5010 5015 5020 5025 5030 5035 5040 5045 5050 5055 5060 5065 5070 5075 5080 5085 5090 5095 5100 5105 5110 5115 5120 5125 5130 5135 5140 5145 5150 5155 5160 5165 5170 5175 5180 5185 5190 5195 5200 5205 5210 5215 5220 5225 5230 5235 5240 5245 5250 5255 5260 5265 5270 5275 5280 5285 5290 5295 5300 5305 5310 5315 5320 5325 5330 5335 5340 5345 5350 5355 5360 5365 5370 5375 5380 5385 5390 5395 5400 5405 5410 5415 5420 5425 5430 5435 5440 5445 5450 5455 5460 5465 5470 5475 5480 5485 5490 5495 5500 5505 5510 5515 5520 5525 5530 5535 5540 5545 5550 5555 5560 5565 5570 5575 5580 5585 5590 5595 5600 5605 5610 5615 5620 5625 5630 5635 5640 5645 5650 5655 5660 5665 5670 5675 5680 5685 5690 5695 5700 5705 5710 5715 5720 5725 5730 5735 5740 5745 5750 5755 5760 5765 5770 5775 5780 5785 5790 5795 5800 5805 5810 5815 5820 5825 5830 5835 5840 5845 5850 5855 5860 5865 5870 5875 5880 5885 5890 5895 5900 5905 5910 5915 5920 5925 5930 5935 5940 5945 5950 5955 5960 5965 5970 5975 5980 5985 5990 5995 6000 6005 6010 6015 6020 6025 6030 6035 6040 6045 6050 6055 6060 6065 6070 6075 6080 6085 6090 6095 6100 6105 6110 6115 6120 6125 6130 6135 6140 6145 6150 6155 6160 6165 6170 6175 6180 6185 6190 6195 6200 6205 6210 6215 6220 6225 6230 6235 6240 6245 6250 6255 6260 6265 6270 6275 6280 6285 6290 6295 6300 6305 6310 6315 6320 6325 6330 6335 6340 6345 6350 6355 6360 6365 6370 6375 6380 6385 6390 6395 6400 6405 6410 6415 6420 6425 6430 6435 6440 6445 6450 6455 6460 6465 6470 6475 6480 6485 6490 6495 6500 6505 6510 6515 6520 6525 6530 6535 6540 6545 6550 6555 6560 6565 6570 6575 6580 6585 6590 6595 6600 6605 6610 6615 6620 6625 6630 6635 6640 6645 6650 6655 6660 6665 6670 6675 6680 6685 6690 6695 6700 6705 6710 6715 6720 6725 6730 6735 6740 6745 6750 6755 6760 6765 6770 6775 6780 6785 6790 6795 6800 6805 6810 6815 6820 6825 6830 6835 6840 6845 6850 6855 6860 6865 6870 6875 6880 6885 6890 6895 6900 6905 6910 6915 6920 6925 6930 6935 6940 6945 6950 6955 6960 6965 6970 6975 6980 6985 6990 6995 7000 7005 7010 7015 7020 7025 7030 7035 7040 7045 7050 7055 7060 7065 7070 7075 7080 7085 7090 7095 7100 7105 7110 7115 7120 7125 7130 7135 7140 7145 7150 7155 7160 7165 7170 7175 7180 7185 7190 7195 7200 7205 7210 7215 7220 7225 7230 7235 7240 7245 7250 7255 7260 7265 7270 7275 7280 7285 7290 7295 7300 7305 7310 7315 7320 7325 7330 7335 7340 7345 7350 7355 7360 7365 7370 7375 7380 7385 7390 7395 7400 7405 7410 7415 7420 7425 7430 7435 7440 7445 7450 7455 7460 7465 7470 7475 7480 7485 7490 7495 7500 7505 7510 7515 7520 7525 7530 7535 7540 7545 7550 7555 7560 7565 7570 7575 7580 7585 7590 7595 7600 7605 7610 7615 7620 7625 7630 7635 7640 7645 7650 7655 7660 7665 7670 7675 7680 7685 7690 7695 7700 7705 7710 7715 7720 7725 7730 7735 7740 7745 7750 7755 7760 7765 7770 7775 7780 7785 7790 7795 7800 7805 7810 7815 7820 7825 7830 7835 7840 7845 7850 7855 7860 7865 7870 7875 7880 7885 7890 7895 7900 7905 7910 7915 7920 7925 7930 7935 7940 7945 7950 7955 7960 7965 7970 7975 7980 7985 7990 7995 8000 8005 8010 8015 8020 8025 8030 8035 8040 8045 8050 8055 8

## 17

comprising at least one metal of the iron group or an alloy thereof, and at least one or both of a solid solution carbide powder of a combination of zirconium and niobium and a solid solution carbonitride powder of a combination of zirconium and niobium;

forming a green compact of said powder mixture; and vacuum sintering or sinter-HIP said green compact at a temperature of from 1400 to 1560° C. wherein the solid solution carbide powder of zirconium and niobium or the solid solution carbonitride powder of zirconium and niobium having a mass ratio  $Nb/(Zr+Nb)$  equal to greater than about 0.5.

2. The method of claim 1 wherein the solid solution carbide powder of zirconium and niobium or the solid solution carbonitride powder of zirconium and niobium having a mass ratio  $Nb/(Zr+Nb)$  greater than or equal to about 0.6.

3. The method of claim 1 wherein the binder metal powder comprises one or more of cobalt powder, nickel powder and iron powder.

4. The method of claim 3 wherein said binder metal powder additionally comprises at least one of chromium and tungsten.

5. The method of claim 1 wherein said binder metal powder comprises between about 3 weight percent and about 15 weight percent of the total mass of said powder mixture.

6. The method of claim 1 wherein said powder mixture additionally comprises at least one carbide, nitride or carbonitride of one or more of titanium, hafnium, vanadium, tantalum, chromium, and molybdenum.

7. The method of claim 1 wherein the total of the solid solution carbide powder of zirconium and niobium and the solid solution carbonitride powder of zirconium and niobium comprises between about 1 weight percent and about 15 weight percent of the total mass of said powder mixture.

8. The method of claim 1 wherein said powder mixture comprises at least one of the elements titanium, hafnium, vanadium, tantalum, chromium and molybdenum in an amount between about 1 weight percent and about 8 weight percent of the total mass of said powder mixture.

9. A method of producing a sintered cemented carbide body comprising the steps of

providing a powder mixture comprising tungsten carbide powder, a binder metal powder comprising at least one metal of the iron group or an alloy thereof, and at least one or both of a solid solution carbide powder of a combination of zirconium and niobium and a solid solution carbonitride powder of a combination of zirconium and niobium; forming a green compact of said powder mixture; and

vacuum sintering or sinter-HIP said green compact at a temperature of from 1400 to 1560° C. wherein the total of the solid solution carbide powder of zirconium and niobium and the solid solution carbonitride powder of zirconium and niobium

## 18

zirconium and niobium comprises between greater than 10 weight percent and about 15 weight percent of the total mass of said powder mixture.

10. A method of producing a sintered cemented carbide body comprising the steps of

providing a powder mixture comprising tungsten carbide powder, a binder metal powder comprising at least one metal of the iron group or an alloy thereof, and at least one or both of a solid solution carbide powder consisting essentially of zirconium and niobium or a solid solution carbonitride powder consisting essentially of zirconium and niobium; forming a green compact of said powder mixture; and vacuum sintering or sinter-HIP said green compact at a temperature of from 1400 to 1560° C. wherein the solid solution carbide powder of zirconium and niobium or the solid solution carbonitride powder of zirconium and niobium having a mass ratio  $Nb/(Zr+Nb)$  equal to greater than about 0.5.

11. A method of producing a sintered cemented carbide body comprising the steps of

providing a powder mixture comprising tungsten carbide powder, a binder metal powder comprising at least one metal of the iron group or an alloy thereof, and at least one or both of a solid solution carbide powder consisting essentially of zirconium and niobium or a solid solution carbonitride powder consisting essentially of zirconium and niobium;

forming a green compact of said powder mixture; and vacuum sintering or sinter-HIP said green compact at a temperature of from 1400 to 1560° C. wherein the solid solution carbide powder of zirconium and niobium or the solid solution carbonitride powder of zirconium and niobium having a mass ratio  $Nb/(Zr+Nb)$  greater than or equal to about 0.6.

12. A method of producing a sintered cemented carbide body comprising the steps of

providing a powder mixture comprising tungsten carbide powder, a binder metal powder comprising at least one metal of the iron group or an alloy thereof, and at least one or both of a solid solution carbide powder consisting essentially of zirconium and niobium or a solid solution carbonitride powder consisting essentially of zirconium and niobium; forming a green compact of said powder mixture; and vacuum sintering or sinter-HIP said green compact at a temperature of from 1400 to 1560° C. wherein the total of the solid solution carbide powder of zirconium and niobium and the solid solution carbonitride powder of zirconium and niobium comprises between greater than 10 weight percent and about 15 weight percent of the total mass of said powder mixture.

\* \* \* \* \*